

## UNITED STATES PATENT OFFICE

CORNELIUS H. KELLER, OF SAN FRANCISCO, CALIFORNIA, ASSIGNOR TO MINERALS SEPARATION NORTH AMERICAN CORPORATION, OF NEW YORK, N. Y., A CORPORATION OF MARYLAND

## ORE CONCENTRATION

No Drawing.

Application filed March 1, 1930. Serial No. 432,562.

This invention relates to flotation concentration of ores and is herein disclosed as applied to the froth flotation of ores with the aid of such a compound as an organic monothio acid or its corresponding disulphide.

5 Such a compound is of the type



wherein R is an organic radical and M is hydrogen or a metal or another



group.

One such compound which is of the ring 15 type, is thio-benzoic acid. This compound was prepared by mixing benzoic acid with about 40% of its weight of phosphorus penta-sulphide and heating to produce a volatile substance which condensed in a receiver 20 to a liquid which finally solidified.

The solid thus collected proved to be a useful agent in connection with a mineral-frothing agent in the concentration of ore. It contained thio-benzoic acid, which was found 25 to be the active principle.

*Example I.*—Utah Copper Company ore was reground with 4 pounds of lime and 0.1 pound of the solid condensate, both per ton of ore, and water, in a ball mill to produce 30 a pulp. The pulp was transferred with additional water to an M. S. subaeration flotation machine and agitated with the addition of 0.1 pound pine oil per ton of ore, and a froth-float concentrate separated. The concentrate thus obtained was put back into the machine and 35 reagitated with the further addition of 0.05 pounds of pine oil per ton of original ore to separate the first concentrate into a finished concentrate and a middling. The results are 40 shown in the following table:

|            | Assays |      | % Recovery |       | 45 |
|------------|--------|------|------------|-------|----|
|            | Cu %   | Fe % | Cu         | Fe    |    |
| Heads..... | 0.968  | 2.93 | 100.0      | 100.0 |    |
| Cones..... | 33.68  | 22.8 | 76.6       | 17.0  |    |
| Midds..... | 2.16   | 4.8  | 10.9       | 7.9   |    |
| Tails..... | 0.13   | 2.4  | 12.5       | 75.1  |    |

50 Another source of a thio acid is pyromucic

or furoic acid, obtained when furfuryl is treated with sodium hydrate to make furfuryl alcohol. This reaction produces furoic acid and furfuryl alcohol.

Thio-furoic acid was produced from furoic acid by mixing the latter with solid phosphorus penta-sulphide and heating to sublime the mixture. The sublimed reaction product contained a substantial proportion of thio-furoic acid. The remainder of the sublimate was principally unchanged furoic acid and contained a small amount of material insoluble in water. Both the thio-furoic acid and the water-insoluble material were found to be useful agents in flotation in connection with mineral-frothing agents.

*Example II.*—Utah Copper Company ore was reground in a ball mill with four pounds of calcium oxide per ton of ore and made into a pulp. The pulp was agitated in the same 70 flotation machine with 0.1 pound of the above-mentioned sublimate and 0.1 pound of pine oil, both per ton of ore, and a froth float concentrate separated. The concentrate thus obtained was put back into the machine and 75 reagitated with 0.05 pound pine oil per ton to separate the first concentrate into a finished concentrate and a middling. The results are shown in the following table:

|            | % wt. | % Cu  | % Fe | Recy. % Cu | % Fe  |
|------------|-------|-------|------|------------|-------|
| Heads..... | 100.0 | 0.95  | 2.88 | 100.0      | 100.0 |
| Conc.....  | 2.3   | 33.44 | 25.2 | 81.1       | 20.1  |
| Midd.....  | 2.5   | 2.60  | 4.6  | 6.9        | 4.0   |
| Tails..... | 95.2  | 0.12  | 2.3  | 12.0       | 75.9  |

*Example III.*—A Tennessee zinc ore from Universal Exploration Company was suitably ground with water to make a pulp and 90 transferred with additional water to a similar flotation machine and agitated with 0.15 pounds of the same sublimate, 0.4 pounds coal tar creosote and 0.1 pounds pine oil, all per ton of ore, and a froth float concentrate separated. The concentrate thus obtained was put back into the machine and agitated with the further addition of 0.05 pounds per tons of the sublimate to separate the first concentrate into a finished concentrate and a

middling. The results are shown in the following table:

| 5          | % wt. | % Zn | Recy.<br>% Zn |
|------------|-------|------|---------------|
| Heads..... | 100.0 | 5.96 | 100.0         |
| Conc.....  | 8.9   | 56.2 | 83.8          |
| Midd.....  | 9.2   | 2.9  | 4.5           |
| Tail.....  | 81.9  | 0.85 | 11.7          |

10 *Example IV.*—A Missouri lead ore from Desloge Consolidated Lead Company was suitably ground with water to make a pulp and transferred with additional water to a 15 similar flotation machine, and agitated with 0.2 pounds of the same sublimate, and 0.1 pounds of pine oil, both per ton of ore, to yield a concentrate and a tailing. The results are shown in the following table:

| 20         | % wt. | % Pb | Recy.<br>% Pb |
|------------|-------|------|---------------|
| Heads..... | 100.0 | 5.63 | 100.0         |
| Conc.....  | 10.38 | 52.0 | 96.0          |
| Tails..... | 89.62 | 0.25 | 4.0           |

30 *Example V.*—Utah Copper Company ore was reground wet in a ball mill for ten minutes with 4 pounds of lime per ton of ore, made 35 into a pulp with additional water and agitated for five minutes with 0.1 pound cresol and 0.05 pounds of the same sublimate, both per ton of ore. A rougher froth concentrate was then separated for five minutes and the 40 tailings were discarded. This rougher concentrate was reagitated for two minutes with the further addition of 0.05 pounds of cresol for two minutes and a finished froth concentrate separated for three minutes. The 45 tailings from this cleaning operation were middlings. The finished concentrate contained 25.92% of copper, the discarded tailings contained 0.10% of copper, so that 78.3% of the copper was recovered in the finished 50 concentrate. Only 25.6% of the iron appeared in the finished concentrate.

With 0.25 pounds of the thio-furoic acid substituted for the amount used in the foregoing procedure, tailings were obtained 55 which contained 0.08% copper, though the grade of concentrate was lower, being 18.95% copper, because of increased iron content.

55 Thio-propionic acid was prepared by heating propionic acid,  $\text{CH}_3\text{CH}_2\text{COOH}$ , with an equal weight of phosphorus pentasulphide and half its weight of coarse sand. From 150 cc. of the propionic acid about 45 cc. of distillate was obtained with a boiling point of 95° to 135° C. On redistillation about 60 half of this distilled at 109° to 112° C.

The latter fraction appeared to consist largely of thio-propionic acid. Part of it was converted into the corresponding disulphide by treatment with potassium ferricyanide. Both the thio-propionic acid and

the corresponding disulphide were found useful in ore concentration.

Thio-acetic acid was found of some value in acid pulps. Thio-salicylic acid was found of some value in pulps made alkaline with lime.

70 Furyl disulphide was made by treatment of a solution of thio-furoic acid with potassium ferricyanide or by treatment of the solution with copper sulphate, which latter procedure concomitantly produced cuprous thio-furoate which precipitated and was separated. This disulphide, produced by either procedure, was found useful in flotation.

75 *Example VI.*—Utah Copper ore was ground with four pounds of lime per ton and made into a pulp and agitated for five minutes with 0.25 pounds of the thio-furyl disulphide and 0.10 pound of pine oil, both per ton of ore, and then a rougher froth concentrate separated for five minutes. The concentrate thus obtained was put back in the machine and reagitated for two minutes with the further addition of 0.05 pound of pine oil per ton, and then a finished concentrate 80 containing 18.44 per cent of copper was separated. This contained 80.1 per cent of the copper of the ore but only 35.3 per cent of the iron. The tailings from this retreatment 85 constitute a middling.

90 *Example VII.*—Utah Cooper Company ore was reground to pass 80-mesh, made into a pulp with water and agitated with 0.25 pounds of the thio-propionic acid, prepared as above described, 0.1 pound pine oil and 95 7 pounds sulphuric acid, all per ton of ore, and a froth-concentrate separated. The heads contained 0.984% copper, the concentrate 11.60% and the tails 0.12% representing a recovery of 88.72%. Nearly as good results were obtained when no acid was added to the pulp, and also when the ore was ground with four pounds of lime per ton.

100 Almost as good results were obtained when, instead of the redistilled thio-propionic acid, there was used, in an alkaline pulp, the residue from the redistillation of the acid or the oily substance extracted with ether from the residue remaining after the preparation of the reaction product.

105 *Example VIII.*—Utah Cooper Company ore was reground to pass 80-mesh, made into a pulp with water and agitated with 0.25 pounds of the disulphide made from thio-propionic acid, 0.1 pine oil, and 7 pounds 110 sulphuric acid, all per ton of ore, and a froth concentrate separated. The heads contained 1.068% copper, the concentrates 16.96% copper, and the tails 0.17%, representing a recovery of 84.93% of the copper.

115 *Example IX.*—Utah Copper Company ore was reground wet with 4 pounds of calcium oxide per ton to pass eighty-mesh and agitated with additional water for two minutes with 0.1 pound of potassium ethyl mono-

thio-carbonate and then 0.2 pounds of cresylic acid were added, both reagents being per ton of ore, and a rougher froth concentrate removed for five minutes. This rougher concentrate was put back into the machine reagitated for two minutes, and then a finished froth concentrate removed for three minutes after the further addition of 0.05 pounds of cresylic acid per ton of original ore. The tailings from this operation constituted a middling. The results are shown in the following table:

| 15     | Assays                       |                                |                             | Insol. | Recoveries                      |                                 |
|--------|------------------------------|--------------------------------|-----------------------------|--------|---------------------------------|---------------------------------|
|        | % wt.                        | % Cu                           | % Fe                        |        | % Cu                            | % Fe                            |
| Cone.  | 100<br>2.81<br>3.82<br>93.37 | 1.012<br>27.68<br>3.20<br>0.12 | 2.90<br>27.2<br>14.3<br>1.7 | 6.5    | 100.<br>76.88<br>12.05<br>11.07 | 100.<br>28.37<br>18.85<br>54.78 |
| Midd.  |                              |                                |                             |        |                                 |                                 |
| Tails. |                              |                                |                             |        |                                 |                                 |

Example X.—Utah Copper Company ore was reground wet with 4 pounds of calcium oxide per ton to pass eighty-mesh and agitated with additional water for two minutes with 0.1 pound potassium amyl mono-thio-carbonate, and then 0.2 pounds cresylic acid was added, both reagents being per ton of ore, and a rougher froth concentrate removed for five minutes. This rougher concentrate was put back into the machine and reagitated for two minutes 0.05 pounds cresylic acid added, and a finished froth concentrate removed for three minutes, the tailings from this operation constituted a middling. The results are shown in the following table:

| 40     | Assays                     |                                |                            |        | Recoveries                     |                                |
|--------|----------------------------|--------------------------------|----------------------------|--------|--------------------------------|--------------------------------|
|        | % wt.                      | % Cu                           | % Fe                       | % Ins. | % Cu                           | % Fe                           |
| Heads. | 100.<br>4.3<br>3.3<br>92.4 | 1.048<br>19.76<br>2.38<br>0.13 | 2.96<br>30.8<br>7.6<br>1.5 | 0.4    | 100.<br>81.11<br>7.44<br>11.45 | 100.<br>44.71<br>8.48<br>44.31 |
| Conc.  |                            |                                |                            |        |                                |                                |
| Midd.  |                            |                                |                            |        |                                |                                |
| Tails. |                            |                                |                            |        |                                |                                |

Example XI.—Utah Copper Company ore was ground wet with 4 pounds of calcium oxide per ton, made into a pulp with 0.1 pound pine oil and 0.25 pound of potassium benzyl mono-thio-carbonate, both per ton of ore, and a froth concentrate separated. The ore contained 1.031% copper, the concentrates 13.12% copper, and the tailings 0.14% copper, representing a recovery of 87.39% of the total copper.

Example XII.—Utah Copper Company ore was ground wet with 4 pounds of calcium oxide per ton, made into a pulp with further water, and agitated with 0.1 pound of pine oil and 0.25 pound potassium butyl mono-thio-carbonate, both per ton of ore, and a froth concentrate separated. The ore contained 1.022% copper, the concentrate 11.92% copper, and the tailings 0.15% copper, representing a recovery of 85.52% of the total copper.

Example XIII.—Utah Copper Company ore was ground wet with 4 pounds of calcium oxide per ton, made into a pulp with further water, and agitated with 0.1 pound of pine oil and 0.25 pound of potassium cyclohexyl mono-thio-carbonate, both per ton of ore, and a froth concentrate separated. The ore contained 1.034% copper, the concentrate contained 12.80% copper, and the tailings 0.12% copper, representing a recovery of 89.26% of the total copper.

It was found that the lead and copper salts of ethyl mono-thio-carbonic acid were effective agents in the flotation concentration of ores.

Example XIV.—Utah Copper Company ore was wet ground to pass eighty-mesh and made into a pulp with water and agitated with 7 pounds sulphuric acid, 0.1 pound pine oil and 0.25 pound of the disulphide made by treating a solution of potassium ethyl mono-thio-carbonate with potassium ferricyanide, all per ton of ore. A froth concentrate was separated containing 11.28% copper. The original ore contained 1.058 copper, and the tailings contained 0.12% copper, representing a recovery of 89.6% of the total copper.

A richer concentrate with nearly as large a recovery was obtained when the sulphuric acid was omitted from the pulp and the ore was ground with calcium oxide before agitation to produce the froth. The disulphide also proved useful in a neutral pulp of the ore.

Having thus described certain embodiments of the invention, what is claimed is:

1. The process of ore concentration which consists in agitating a pulp of an ore with an organic compound containing the group



in which R is an organic group and M is hydrogen or a metal or another



group, so as to form a floating concentrate, and separating the float.

2. The process of ore concentration which consists in agitating a pulp of an ore with an organic compound containing the group



in which R is a cyclic, organic group, and M is hydrogen or a metal or another



group, so as to form a floating concentrate, and separating the float.

3. The process of ore concentration which

consists in agitating a pulp of an ore with an organic compound containing the group



- 5 in which R is an organic group connected to the carbon atom by a carbon atom of the R group, and M is hydrogen or a metal or another

10



group, so as to form a floating concentrate, and separating the float.

4. The process of ore concentration which 15 consists in agitating a pulp of an ore with a non-nitrogenous mono-thio derivative of an organic acid in which the double-bonded oxygen and the sulphur are attached to the same carbon atom, the agitation being conducted 20 under such conditions that a floating concentrate is formed, and separating the float.

5. The process of ore concentration which consists in agitating a pulp of an ore with a mono-thio derivative of a cyclic, organic acid 25 in which the double-bonded oxygen and the sulphur are attached to the same carbon atom, the agitation being conducted under such conditions that a floating concentrate is formed, and separating the float.

- 30 6. The process of ore concentration which consists in agitating a pulp of an ore with a mono-thio derivative of furoic acid in which the double-bonded oxygen and the sulphur are attached to the same carbon atom, the agitation being conducted under such conditions that a floating concentrate is formed, and separating the float.

- 35 7. The process of ore concentration, which consists in agitating a pulp of an ore with 40 a compound having the formula



- 45 in which R stands for the furyl group under such conditions that a floating concentrate is formed, and separating the float.

8. The process of ore concentration which 50 consists in grinding the ore in a pulp containing a non-nitrogenous mono-thio organic acid and thereafter agitating the ore pulp in the presence of a mineral-frothing agent so as to concentrate the mineral as a float, and separating the float.

In testimony whereof, I have affixed my 55 signature to this specification.

CORNELIUS H. KELLER.